

Patented Dec. 15, 1931

1,836,400

# UNITED STATES PATENT OFFICE

AUGUST RUPPERT, OF FRANKFORT-ON-THE-MAIN, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## MANUFACTURE OF SOAPS

No Drawing. Application filed November 12, 1928, Serial No. 319,013, and in Germany November 15, 1927.

This invention relates to the manufacture of soaps which are especially adapted for dissolving fats, oils, resins and contaminations of any kind. For this purpose it has been proposed to incorporate chlorinated hydrocarbons in a water-soluble form into soap, and such preparations which are put up for sale in the form of liquids have been used to a great extent in textile industries. However, they have not been adopted in households and workshops for the following reasons.

First of all the intense smell of the preparations when used for domestic purposes has been objected to; secondly such preparations could not be utilized for washing and cleaning purposes owing to their property of excessively extracting the fat from the skin, and thirdly the liquid form in which the preparations were hitherto prepared often impeded their general use.

Now I have found that excellent products of the kind referred to are obtained by incorporating into soap water-soluble monoalkyl ethers of the group comprising glycols and polyglycols, as for instance, diethylene-glycol, triethyleneglycol and mixtures thereof. For instance, by admixing glycolmonoalkylethers  $C_nH_{2n-1}OH. OR$  (for instance, an ethylene-, propylene- or butylene-glycol-ether) or ethers of polyethyleneglycols, which are good solvents for certain substances, such as fatty oils of vegetable or animal origin or mineral oils and resins, soda or potash soaps are obtained having an increased cleaning capacity. The said ethers are soluble in water and this property also belongs to the aqueous solutions of such soaps.

A further advantage consists in that no sensible change of smell is imparted to the new soaps by the incorporation of the said ethers which themselves have only a slight aromatic odour.

Potash soaps are easily soluble in glycolmonoalkylethers; their solubility is increased by a small addition of water. Therefore glycolmonoalkylethers may be mixed within wide limits with varying amounts of potash soaps to form liquid or jelly-like products.

Soda soaps are, as a rule, rather difficultly soluble in the liquid glycolmonoalkylethers when cold; they are more soluble at temperatures from about 50° to 100° C. In this case the solubility may also be increased by a slight addition of water. Even with a small percentage of soap, amounting to about 10% or less, the mixture solidifies forming gelatinous, transparent products. By increasing the percentage of soda soap and treating the mixture at temperatures from 50° to 100° C. with the addition of small quantities of water transparent soaps of remarkable hardness are obtained on cooling down.

I have further found that the presence of the said glycol- or polyglycolethers in the soap facilitates the incorporation of numerous other fat-solvents, such as liquid hydrocarbon compounds, including their halogen substitution products as, for instance, chlorinated hydrocarbons of the aliphatic, aromatic or hydroaromatic series. By varying the proportions of the ingredients (including water) either solid or jelly-like or unguentary products may be obtained.

For producing the new soap I may proceed in such a way that the soda or potash soap or the soap-paste is first stirred with the glycolether at temperatures from about 50° to 100° C. and then the other ingredients are added in a closed vessel, stirring and heating being continued. Thereafter the mass is allowed to solidify or to gelatinize, as the case may be.

In all cases the said glycolethers or polyglycolethers and the liquid hydrocarbon compounds may be added to the finished soaps, or the ethers and, if desired, also the other ingredients or mixtures or both may be added or incorporated to the raw materials from which the soap is produced. The final products are distinguished by the same qualities as the products obtained by adding the same ingredients to the finished soap, but are especially characterized by their strong frothing or lathering power and by their agreeable action upon the skin.

As ascertained by experiments, the above-named ethers are not attacked, when present

while the process of saponifying oils or fats is performed. Preferably I may proceed in such a way that the fat or oil to be saponified is first dissolved in the ether to be employed, 5 then the saponification is effected and thereafter, if desired, a liquid hydrocarbon or a liquid chlorinated hydrocarbon is added. In some cases it may be advantageous to mix the fat or oil to be saponified with the ether along 10 with the hydrocarbon or chlorinated hydrocarbon and then to subject the mixture to saponification.

Owing to the fact that glycolalkylethers have a higher boiling point than the liquid 15 hydrocarbons or chlorinated hydrocarbons employed, the former perform the action of decreasing the vapor tension of the latter whereby the smell of the preparations is reduced to such a degree that it is no longer 20 perceived as offensive when using the products. The slight proper odour of the ethers does not appear at all.

Being liquids of a slightly oily character which are easily soluble in water as well as 25 in hydrocarbons and chlorohydrocarbons, the glycolalkylethers and the (individual or mixed) polyglycolalkylethers are furthermore characterized by the fact that they largely repress the feeling of fat-extracting 30 from the skin. Indeed the properties of soaps even containing, for instance, more than 30% of chlorinated hydrocarbons are altered to such an extent that no roughness or hardness of the skin is brought about, but on the contrary 35 the skin gets a soft, tender and pliable character which is preserved unchanged even after repeated washing. As compared with glycerine soaps, the new soaps are distinguished by a superior cleaning power, as 40 glycerine is no solvent for fatty oils, resins and the like.

One of the advantageous results produced by the addition of glycol- or polyglycolalkylethers to soda or potash soap consists in that 45 considerable quantities of liquid hydrocarbon compounds as defined above, according to the requirements of the practice, can be incorporated into the soap without the said hydrocarbon compounds etc. being separated on 50 dilution with water. Furthermore the essential fact has been ascertained that, with the aid of the above-said ethers, from 30 to 40% of liquid hydrocarbon compounds, as will be shown by the examples may be incorporated 55 into potash soaps or mixed soda and potash soaps without the tough, jelly-like appearance of the soft soaps being altered. By adding a higher percentage of ethers and hydrocarbon compounds or water unguentary or 60 liquid, products are obtained, the action of which on the skin is likewise agreeable and irreproachable.

Soda soaps may be produced according to 65 my invention and pressed into moulds.

### Examples

1. 250 parts of soft soap are, at temperatures from about 50° to 100° C. mixed, while stirring, with 40 parts of glycolmonobutyl- 70 ether, and, while further stirring, 200 parts of carbon tetrachloride are added. The appearance of the soft soap remains unaltered. On dissolving the product in water, no carbon tetrachloride is separated.

2. 50 parts of hard soap and 200 parts of soft soap are first mixed and heated to form a uniform paste. Thereupon 40 parts of glycolmonomethylether are added while stirring and continued heating and then 200 parts of carbon tetrachloride are introduced, stirring 80 being continued. A tough, jelly-like soft soap is obtained. On adding water, no part of the chlorohydrocarbon is separated.

3. 250 parts of soda soap paste are mixed, 85 while stirring with 40 parts of glycolmono-ethylether. Then 200 parts of carbon tetrachloride are introduced, likewise while stirring at temperatures from about 50° to 100° C. After cooling-down the product 90 solidifies in the form of a tough paste, from which on mixing with water the chlorinated hydrocarbon does not separate.

4. 240 parts of bleached linseed oil are mixed, while stirring with 100 parts of water on the water-bath to form a fine emulsion. Then 54 parts of caustic potash dissolved in 100 parts of water are gradually added while stirring. The stirring is continued; further quantities of water being 100 added until the saponification is completed. The water then amounts to 470 parts. Thereupon 80 parts of glycolmonoethyl-ether and then 360 parts of carbontetra- 105 chloride are added while further stirring. A creamlike soap is obtained.

5. 250 parts of soft soap, 40 parts of glycolmonobutylether and 115 parts of toluene are mixed while stirring at room temperature. A jelly-like mass is produced having 110 the appearance of common soft soap.

6. 200 parts of hard soap are dissolved, while stirring in a hot solution of 100 parts of glycolmonoethylether and 30 parts of water; then the mixture is cooled down to 115 some extent and 95 parts of tetraline are added. On cooling down, the mass solidifies as a transparent solid soap.

7. 200 parts of hard soap are dissolved at temperatures from about 50° to 100° C. in a mixture of 100 parts of glycolmonoethyl-ether and 30 parts of water while stirring; then the mixture is cooled down to some extent and 75 parts of benzine are added while stirring. On cooling down the mass solidifies 125 in the form of a hard soap.

Instead of potash or soda soaps a mixture of both may be used.

8. 240 parts of linseed oil are mixed with 80 parts of glycolmonoethylether. The 130

- mixture is now saponified with 54 parts of caustic potash dissolved in 81 parts of water while heating. The soap is mixed when still hot with 180 parts of carbontetrachloride. 5 A product is obtained having the appearance of a jelly-like soft soap. 9. 100 parts of cocoa-nut fat are dissolved in a mixture of 60 parts of glycolmonoethyl-ether and 90 parts of carbontetrachloride. 10 Then the fat is saponified with 52 parts of a hot caustic soda solution showing 38° Bé. On cooling-down, the product solidifies as a hard soap. 10. 240 parts of linseed oil are mixed with 15 100 parts of glycolmonobutylether. The mixture is then saponified with 54 parts of caustic potash dissolved in 31 parts of water while heating. A jelly like soap is obtained having the appearance of soft soap. 20 The product may be mixed, if desired, with 120 parts of tetraline, benzine or toluene. 11. 100 parts of cocoa-nut fat are dissolved in a mixture of 60 parts of glycolmonoethyl-ether and 70 parts of tetraline. Then the 25 fat is saponified with 52 parts of a caustic soda solution of 38° Bé while heating. On cooling-down, the product solidifies as a hard soap. 12. 100 parts of cocoa-nut fat are dissolved 30 in a mixture of 60 parts of glycolmonoethyl-ether and 60 parts of toluene. Then the fat is saponified with 52 parts of a caustic soda solution of 38° Bé while heating. After cooling-down, the mixture solidifies as a 35 hard soap. 13. 100 parts of cocoa-nut fat are dissolved in a mixture of 60 parts of glycolmonoethyl-ether and 60 parts of benzene. The fat is saponified with 52 parts of a caustic soda 40 solution of 38° Bé while heating. After cooling down, the mixture solidifies as a hard soap. 14. 240 parts of linseed oil are mixed with 100 parts of the monoethylether of a technical 45 mixture of polyethyleneglycols. Then the mixture is saponified at temperatures from about 50° to 100° C. with 54 parts of caustic soda dissolved in 81 parts of water; thereupon 180 parts of carbontetrachloride 50 are added while stirring. A product is obtained having the appearance of a jelly-like soft soap. 15. 200 parts of hard soap are dissolved in 100 parts of monoethylether of mixed poly- 55 ethyleneglycols while heating. After cooling-down, the product solidifies forming a hard soap. 16. 100 parts of monoethylether of mixed polyethyleneglycols are dissolved at tem- 60 peratures from about 50° to 100° C. in 400 parts of soft soap. By adding to the clear solution 150 parts of tetraline, a jelly-like soft soap is produced. 17. 400 parts of soft soap are dissolved at 65 temperatures from about 50° to 100° C. in 100 parts of monoethylether of mixed polyethyleneglycols and 210 parts of benzine are added to the clear solution. A liquid soap is obtained. 18. 400 parts of soft soap are dissolved at 70 temperatures from about 50° to 100° C. in 100 parts of monoethylether of mixed polyethyleneglycols and to the clear solution 150 parts of toluene are added. A jelly-like soft soap is obtained. 75 It will be understood that the term "hydrocarbon compound" wherever it occurs in the following claims is to include those hydrocarbons and their halogen substitution products which are in common use as volatile 80 solvents. 85 I claim:—
  - As a new article of manufacture and trade, a soap containing a monoalkylether of the group comprising glycols and polyglycols and a liquid chlorinated hydrocarbon.
  - As a new article of manufacture and trade, a soap containing a monoalkylether of the group comprising glycols and polyglycols and carbon tetrachloride.
90 In testimony whereof, I affix my signature.
- AUGUST RUPPERT.
- 95
- 100
- 105
- 110
- 115
- 120
- 125
- 130